

# UNITED STATES PATENT OFFICE.

MAX BECKE, OF HÖCHST-ON-THE-MAIN, GERMANY, ASSIGNOR TO FARBWERKE VORM. MEISTER LUCIUS & BRÜNING, OF HÖCHST-ON-THE-MAIN, GERMANY, A CORPORATION OF GERMANY.

## PROCESS OF PRODUCING MULTICOLORED EFFECTS IN SPUN AND WOVEN GOODS.

1,002,118.

Specification of Letters Patent.

Patented Aug. 29, 1911.

No Drawing.

Application filed July 18, 1910. Serial No. 572,637.

To all whom it may concern:

Be it known that I, MAX BECKE, engineer-chemist, a citizen of the Empire of Germany, residing at Höchst-on-the-Main, Germany, have invented certain new and useful Improvements in Processes of Producing Multicolored Effects in Spun and Woven Goods, of which the following is a specification.

- 10 In U. S. Patent No. 815,671 is described a process for modifying the affinity of wool fiber for dyestuffs in such a manner that multi-colored effects of any kind can be obtained in dyeing fabrics composed entirely 15 or partly of wool. Hitherto no analogous process for producing such effects on vegetable fiber has been known. Now I have found that similar white or colored effects 20 can be produced in dyeing cotton and other vegetable material by applying, on the one hand, the oxidizing action of the higher ox- 25 ides of manganese upon certain dyestuffs, and on the other hand, the stability of cer- 30 tain cotton dyestuffs to this oxidizing action. According to the new method the proce- 35 dure is as follows: The cotton (loose cotton, laps, yarns or twisted yarn) to be rendered capable of resisting dye is prepared with higher oxides of manganese. For this purpose 40 it is impregnated with a concentrated solution of a salt of peroxid of manganese, for exam- 45 ple manganous chlorid. It is then treated with a strongly-alkaline solution, for exam- 50 ple one of caustic soda or ammonia, whereby a manganese hydroxid is precipitated on the fiber. An active oxidizing agent such as a 55 hypochlorite or chromate is usually added to this alkaline bath to effect the formation of the insoluble higher oxides of manganese. 60 Or in lieu of such addition, the manganous hydroxid precipitated by the alkaline solution may be transformed into the higher ox- 65 ids on the fiber, by the absorption of atmos- 70 pheric oxygen when drying. The essential 75 feature of the process is the provision on the fiber of higher manganese oxides, whether the sesquioxide or the dioxide, which act in 80 the final stage to liberate oxygen in the acid dye-bath and thereby destroy the ground- 85 dyestuff at the prepared spots. For the pro- 90 duction of color effects contrasting with those of the subsequent dyeing, the cotton or other vegetable fiber must be dyed with dye- 95 stuffs which are fast to oxidizing agents

(thioindigo derivatives, anthraquinone, vat- 55 dyestuffs, insoluble azo-dyestuffs or the like) before it is impregnated with the manganese salt. The white or colored vegetable fibers thus prepared with higher oxides of manga- 60 nese are used together with undyed cotton or another vegetable fiber or an animal fiber for manufacturing spun goods and woven goods. These spun goods and woven goods can, if required, be steeped, washed, boiled 65 in the kier bleached or mercerized before the dyeing, without detriment to the action of the oxides of manganese. If the fabrics and spun goods thus prepared are then dyed, the dyestuffs used, so far as they are substantive 70 cotton dyestuffs, are absorbed by the treated and untreated fibers. However, if the dyed material is passed through an acid bath, and if for the second dyeing the proper dyestuffs are used, the color absorbed in the second 75 bath is removed from those parts of the fiber which are loaded with the manganese oxides; after the passage through the acid bath it is 80 advantageous to pass the material through a bath of oxalic acid, bisulfite or the like. In this manner a fabric of any ground-color 85 decorated with white or colored effects is obtained. For the dyeing in the second bath there can be used, among other dyestuffs, substantive cotton - dyestuffs, azo - dyestuffs capable of being diazotized, and indigo. 85

The resulting spun and woven goods hav- 90 ing multi-colored effects are characterized by the fact that their ground-color is de- 95 stroyed when treated with a hypochlorite solution of 1-2° Twaddle, while the multi- colored effects withstand this treatment.

The great technical advantage of the pres- 95 ent process consists in the possibility of 100 keeping the current patterns in stock and dyeing them any ground color, as and when required.

In calico printing the production of re- 105 sist and discharge effects on indigo-dyed goods by means of the higher oxides of man- ganese and acids is known; however, a great number of the usual resist, discharge and printing processes cannot be applied in multi-colored dyeing. Moreover the piece dyeing of fabrics consists of vegetable fiber with colored effects, has not yet been carried out in practice, whereas this problem has already been solved as regards wool fiber in an excellent manner, according to U. S. Patent

No. 815,671. The possibility of industrially producing contrast-effects of any tint in dyeing vegetable fibers in the piece was not, therefore, to be foreseen.

5 Having now described my invention, what I claim is:

1. The herein described process of producing multicolored effects in spun and woven goods, by precipitating on vegetable fibers manganese oxids, then working the fibers thus treated together with untreated fibers, dyeing the goods thus manufactured, and subsequently treating the goods with agents capable of developing the oxidizing action of the manganese oxids.
- 10 2. The herein-described process of pro-

ducing multi-colored effects in spun and woven goods, by precipitating on the vegetable fibers dyed with dyestuffs resisting oxidizing agents, manganese oxids, then working the fibers thus treated together with untreated fibers, dyeing the goods thus manufactured, and subsequently treating the goods with agents capable of developing the oxidizing action of the manganese oxids. 20 25

In testimony whereof, I affix my signature in presence of two witnesses.

MAX BECKE.

Witnesses:

JEAN GRUND,  
CARL GRUND.

---

Copies of this patent may be obtained for five cents each, by addressing the "Commissioner of Patents, Washington, D. C."

---